

Oct. 27, 1970

F. D. HESS

3,536,543

NONCORROSIVE NITROGEN TETROXIDE CONTAINING  $P_2O_5$

Filed April 3, 1968



CORROSION RATES FOR MAGNESIUM IN  
NITROGEN TETROXIDE  
 $NH_4 PF_6$  AND  $P_2 O_5$  INHIBITORS

INVENTOR.

FRANK D. HESS

BY

Harry A. Herbert Jr.  
William J. O'Brien  
ATTORNEYS

1

3,536,543

## NONCORROSIVE NITROGEN TETOXIDE CONTAINING $P_2O_5$

Frank D. Hess, Malibu, Calif., assignor to the United States of America as represented by the Secretary of the Air Force

Filed Apr. 3, 1968, Ser. No. 718,610  
Int. Cl. C01b 21/36; C06d 5/08

U.S. Cl. 149—74

2 Claims

### ABSTRACT OF THE DISCLOSURE

A method for the facile control of the corrosive effects produced on metal surfaces by water-bearing nitrogen tetroxide. The method involves adding sufficient amounts of phosphorus pentoxide to the water-bearing nitrogen tetroxide as a corrosion inhibiting additive. The water content of the nitrogen tetroxide preferentially reacts with the phosphorous pentoxide inhibitor to form phosphoric acid instead of reacting with the nitrogen tetroxide to form nitric acid. This preference results in minimizing the quantity of corrosive nitric acid formed and allows the resulting phosphoric acid to react with the surface of the tank to form a protective metal phosphate film.

### BACKGROUND OF THE INVENTION

This invention relates to a method for inhibiting the corrosion of metal surfaces by nitrogen tetroxide. In a more specific manner, this invention concerns itself with nitrogen tetroxide rocket fuel oxidizers containing small amounts of water and to a method for protecting metals from the corrosive effect of such oxidizers through the utilization of a phosphorus pentoxide corrosion inhibiting additive.

The recent advent of nitrogen tetroxide as an oxidizer for liquid propellant rocket fuels has created a materials handling problem of major proportions. Its storage and handling has been attended by corrosion problems and metal failure especially at the welds of aluminum storage containers. Corrosion failure is caused by the presence of water in the nitrogen tetroxide oxidizer and is enhanced by the affinity of the oxidizer for atmospheric moisture.

No corrosion problem has been encountered when using anhydrous nitrogen tetroxide. This is borne out by the fact that tests have shown anhydrous nitrogen tetroxide is practically noncorrosive and that when water content is held within specified limits, ordinary chemical-corrosion failures do not occur. Accordingly, military procurement specifications for water in nitrogen tetroxide limits its concentration to 0.1 weight percent of the material as procured, and under field conditions, water concentration is not allowed to exceed 0.2 weight percent water.

In practice, however, experience has shown that contamination of nitrogen tetroxide by water is difficult to avoid because of its inherent hygroscopic nature as well as the circumstance that it is frequently stored at temperatures below ambient, thus producing local condensation of moisture in the interior of storage tanks and transfer lines. Prior to this invention, no known methods were available for the facile control of corrosion by wet nitrogen tetroxide. Consequently, corrosion failure of storage tanks with the attendant exposure of personnel to the highly toxic effects from this material constituted an ever present danger whenever the oxidizer was utilized in aerospace operations.

One of the primary drawbacks found to exist during attempts to overcome the corrosive effect of wet nitrogen tetroxide was the low solubility in nitrogen tetroxide of inhibitors commonly used in other corrosive liquids. Also,

2

it had been observed that inadequate amounts of so-called inhibitors may actually promote corrosion. Many inorganic inhibitors such as chromates, arsenates and iodates were found to be ineffective in nitrogen tetroxide because of their low solubility in this nonpolar material. Organic inhibitors, such as amines, were, in general, found to be incompatible with nitrogen tetroxide. The discovery of a good corrosion inhibitor for nitrogen tetroxide therefore, became a problem of the highest practical interest.

With this invention, however, the problems encountered in using moist nitrogen tetroxide as an oxidizer for rocket fuels have been abrogated to a great degree through the discovery that phosphorus pentoxide functions as an efficient and effective corrosion inhibiting additive for water-bearing nitrogen tetroxide. While nearly insoluble in anhydrous nitrogen tetroxide, phosphorus pentoxide will dissolve to form phosphoric acid to the extent that water is present, thus restoring the moist nitrogen tetroxide to its noncorrosive condition.

### SUMMARY OF THE INVENTION

In accordance with the present invention, it has been found that the corrosive effect produced on metal surfaces by moist nitrogen tetroxide can be easily controlled in an effective manner by using phosphorus pentoxide as a corrosion inhibiting additive. The inhibitor reacts with the water present in the nitrogen tetroxide to form phosphoric acid thus causing the water containing nitrogen tetroxide to revert to its noncorrosive anhydrous state. Consequently, the problem of metal surface corrosion attendant with the use of nitrogen tetroxide as a liquid propellant oxidizer has been largely overcome.

Accordingly, the primary object of this invention is to provide a method whereby the corrosion of metal surfaces by wet nitrogen tetroxide is substantially eliminated.

Another object of this invention is to provide a corrosion inhibiting additive for nitrogen tetroxide.

Still another object of this invention is to provide a corrosion inhibited nitrogen tetroxide oxidizer for rocket fuels which is adapted to adequately protect the metal surfaces of storage containers from the corrosive effects of a water-nitrogen tetroxide system.

A further object of this invention is to provide a method for inhibiting the corrosion of metal surfaces in a relatively simple, yet effective manner.

These and still further objects and advantages of this invention will become readily apparent from the description of the invention which follows when taken in conjunction with the accompanying drawing.

### DESCRIPTION OF THE DRAWING

In the drawing:

The figure presents a graphical illustration pointing out the effectiveness of the corrosion inhibiting additive of this invention.

### DESCRIPTION OF THE PREFERRED EMBODIMENT

Pursuant to the objects of this invention, the present method involves the addition of phosphorus pentoxide to moist nitrogen tetroxide. The phosphorus pentoxide functions as a corrosion inhibiting additive thereby permitting the facile utilization of nitrogen tetroxide as a rocket fuel oxidizer. The inhibitor may be added to the oxidizer supply tank of a bipropellant fuel system and the fuel may be selected from any of those conventionally used such as monomethylhydrazine (MMH) or a blend of hydrazine and unsymmetrical dimethylhydrazine (UDMH). The manner in which the inhibitor is added to the nitrogen tetroxide oxidizer is not critical and any conventional

filling means can be employed. No particular equipment or safeguards are essential.

The amount of inhibitor needed to control the corrosive nature of moist nitrogen tetroxide depends on the amount of water present in the tetroxide since the phosphorus pentoxide will react to form phosphoric acid to the extent that water is present. More specifically, the present military procurement specifications permit the presence of not more than 0.1 weight percent water in nitrogen tetroxide oxidizers. As a consequence, one pound of phosphorus pentoxide is required per 32 gallons of nitrogen tetroxide to prevent corrosion with this percentile of water.

In order to evaluate the effectiveness of the inhibitor, a resistance testing method was utilized. The changing resistance of a magnesium ribbon in a corrosive medium,  $N_2O_4$  plus 0.5 weight percent  $H_2O$  and various inhibitors, was measured as a function of time. Three typical curves: (1)  $NH_4PF_6$ , (2)  $P_2O_5$  and  $H_2O$  with inhibitor, and (3)  $P_2O_5$  and  $H_2O$  without inhibitor, are illustrated in the figure of the drawing. They have the general form:

$$\sigma \log x = \log y \quad (1)$$

where  $\sigma$ , the slope of the curve, is a measure of the corrosion rate. The smaller the value of  $\sigma$ , the greater is the corrosion protection. The values of the inhibitors tested are given in Table I.

Use of this slope in devising a figure of merit for rating inhibitors requires a second factor, the intercept of the curve on the Y-axis. This intercept should have a low value if corrosion inhibition is effective. Compensation is made for variation in the initial resistance of the test strips by an equivalent figure, which is obtained graphically by determination of the time at which the resistance of the test strip has increased 2%. The final figure of merit is the ratio of the quotient of this time divided by the slope of the curve and the same quotient for water without an inhibitor:

$$FM = \frac{T_i/\sigma_i}{T_w/\sigma_w} \quad (2)$$

where  $FM$  = figure of merit;  $T_i$  = time for 2% resistance increase, inhibitor added;  $\sigma_i$  = slope of corrosion rate curve from Table I;  $T_w$  = time for 2% resistance increase, no inhibitor; and  $\sigma_w = 0.56$ , slope of corrosion rate curve for water.

TABLE I

Corrosion protection of magnesium by inhibitors

| Inhibitor:          | $\sigma$ |
|---------------------|----------|
| $P_2O_5$            | 0.28     |
| $NH_4PF_6$          | 0.33     |
| $H_3PO_4$           | 0.37     |
| $As_2O_3 + Sb_2O_3$ | 0.38     |
| $KIO_3$             | 0.38     |
| $As_2O_3$           | 0.40     |
| $H_2SO_4$           | 0.40     |
| $KIO_4$             | 0.44     |
| $KI$                | 0.47     |
| $I_2$               | 0.48     |
| No inhibitor        | 0.56     |

It is apparent from Table II that  $P_2O_5$  has a real value in protecting magnesium from corrosion by water-bearing  $N_2O_4$ .  $P_2O_5$  is a powerful desiccant and is more likely to act by forming phosphoric acid with the water in preference to the formation of nitric acid. This preference results in minimizing the quantity of corrosive  $HNO_3$ .

formed. The resulting  $H_3PO_3$  reacts with the surface of the metal to form a protective metal phosphate film.

In the figure of the drawing, the curves plotted for corrosion of magnesium with no inhibitor and with  $P_2O_5$  inhibitor have a low initial slope, as indicated by the dashed portion of the curve. This low initial slope was noted in most tests and may represent a period of slow removal of an oxide coating from the magnesium.

TABLE II

Figure of merit for inhibitors with magnesium

| Inhibitor:          | Figure of merit |
|---------------------|-----------------|
| $P_2O_5$            | 190.00          |
| $KI$                | 1.43            |
| $KIO_4$             | 1.42            |
| $KIO_3$             | 1.33            |
| $As_2O_3$           | 1.33            |
| $H_3PO_4$           | 1.09            |
| $As_2O_3 + Sb_2O_3$ | 1.09            |
| $I_2$               | 1.08            |
| No Inhibitor        | 1.00            |
| $H_2SO_4$           | 0.90            |
| $NH_4PF_6$          | 0.34            |

From the foregoing description it will be apparent that this invention provides a method which is most effective in controlling the deterioration of metal surfaces from the corrosive effect of moist nitrogen tetroxide. The utilization of the phosphorus pentoxide inhibitor of this invention has unexpectedly facilitated the use of nitrogen tetroxide as an oxidizer for rocket fuels and has enabled those skilled in the field to take practical advantage of the desirable oxidizing properties of nitrogen tetroxide.

The invention has been described with particular reference to a specific embodiment thereof. It is to be understood, however, that the description of the present invention is for the purpose of illustration only and is not intended to limit the invention in any way, the scope of which is defined by the appended claims.

What is claimed is:

1. A method for inhibiting the corrosive action produced on metal surfaces by water-bearing nitrogen tetroxide which comprises adding phosphorus pentoxide to said nitrogen tetroxide in an amount sufficient to effect a preferential reaction between said phosphorus pentoxide and said water to the extent that water is present in the water-bearing nitrogen tetroxide.

2. A method in accordance with claim 1 wherein about one pound of phosphorus pentoxide is added to about thirty-two gallons of a nitrogen tetroxide solution bearing 0.1 weight percent water.

## References Cited

## UNITED STATES PATENTS

2,403,932 7/1946 Lawson ----- 149—74 XR  
3,383,859 5/1968 Croomes ----- 60—214

## FOREIGN PATENTS

476,227 12/1937 Great Britain.

## OTHER REFERENCES

Ross, Journal American Rocket Society, No. 80, March 1950, pp. 24—31, 149—74, Lit. No. TL788A8.

65 BENJAMIN R. PADGETT, Primary Examiner

U.S. CL. X.R.

23—157; 149—109